

# UNITED STATES PATENT OFFICE.

W. A. OTTO WUTH, OF PITTSBURG, PENNSYLVANIA.

## METHOD OF REMOVING SILICON FROM WROUGHT-IRON.

SPECIFICATION forming part of Letters Patent No. 311,159, dated January 20, 1885.

Application filed June 2, 1884. (No specimens.)

*To all whom it may concern:*

Be it known that I, W. A. OTTO WUTH, of Pittsburgh, in the county of Allegheny and State of Pennsylvania, have invented a new 5 and useful Improvement in Methods of Removing Silicon from Wrought-Iron; and I do hereby declare the following to be a full, clear, and exact description thereof.

It is of great importance that the iron used 10 in the manufacture of crucible and the better grades of open-hearth steel should be as free as possible from silicon, whether chemically combined with it or in the shape of slag, cinder, or silicate of iron. It is also essential 15 for the manufacture of good steel that the percentage of silicon in the iron should be uniform. The amount of chemically-combined silicon is, as a rule, very small, while the percentage of slag in blooms or billets—in 20 which shapes the iron is generally supplied to the steel-manufacturers—I have found to vary usually from one to two and one-half per cent., and sometimes as high as four per cent. One per cent. of slag contains about .12 per 25 cent. of silicon, and 2.50 per cent. of slag .30 per cent. of silicon.

The iron as it comes from the furnace to be hammered into blooms or billets, no matter by what process produced—the Catalan forge 30 or puddling-furnace—consists of a spongy, pasty mass of iron the interstices of which are filled with a fluid slag or cinder, (silicate of iron.) The separation of the slag from iron is accomplished by mechanical means. For the 35 lower grades of iron, not suitable for making steel, it is done by passing the balls through a squeezer, and in other cases by hammering. If, when the balls are at a white heat, so that the cinder is limpid like water, the full force of 40 the hammer could be applied immediately, all or nearly all of the cinder could be driven out, leaving the iron comparatively free from slag. But in practice this cannot be done, as it would cause the iron to scatter in all directions, which would be both dangerous and wasteful. The practice, therefore, is to begin 45 with light blows, delivered on all sides of the ball, which is frequently turned, until the iron becomes gradually solid enough to allow the

full force of the hammer to be applied. Nearly 50 one-half of the time necessary to reduce the ball to a solid billet or bloom is occupied in getting it solid enough to allow of the full force of the hammer. During this process of hammering the slag becomes too pasty to be completely separated from the iron. Just in proportion as the temperature of the ball is allowed to become lower and the slag more pasty will the bloom or billet contain more or less slag, the silicon of which in contact 60 with the carbon in the crucible, reduced from silicic acid in the slag to silicon, combines with the iron, and the result is steel with varying percentages of silicon. One hammer is provided for several furnaces, and as the 65 balls, after being formed, cannot be kept in the furnace without oxidizing part of the iron, they often have to be taken out and kept in the air when the hammer is occupied. This allows them to cool before reaching the 70 hammer, so that the iron is too solid and the slag too pasty to permit the latter to be driven out, no matter how perfectly the hammering is done.

My improved process of freeing the ball 75 from the slag, and thereby obtaining a better and more regular product, is as follows: I take the ball as soon as it comes from the furnace and pass it through the squeezer, by preference the rotary one, which makes it 80 sufficiently solid to receive the full force of the hammer. It is now too cold to enable the slag to be eliminated by hammering. I therefore take it after it comes from the squeezer, and with or without passing it through the 85 so-called "muck-rolls," by preference without, to a reverberatory furnace, and submit it to a neutral or but slightly-oxidizing flame, and, after bringing it to a white heat, remove it from the furnace and hammer the now liquid 90 cinder out of the porous mass of iron.

By the practical use of my invention I have, under unfavorable circumstances, produced blooms containing only from .06 to .07 per cent. of silicon, while the best Lake Champlain blooms contain from .12 to .30 per cent.

I do not claim the squeezing, heating, or hammering of iron balls, separately; but

What I do claim as my invention, and desire to secure by Letters Patent, is—

The improved method of removing silicate of iron from wrought-iron, which consists in 5 passing the heated ball as it comes from the furnace through the squeezer, then reheating, and finally hammering it, substantially as described.

In testimony whereof I have hereunto set my hand this 29th day of May, A. D. 1884.

W. A. OTTO WUTH.

Witnesses:

JOS. H. JACOBS,  
J. K. SMITH.